

Oct. 10, 1944.

M. F. FILLIUS

2,360,216

SUBBING PHOTOGRAPHIC PAPER SUPPORTS

Filed June 8, 1943

FIG. 1.



FIG. 2.



MILTON F. FILLIUS

INVENTOR

BY *Milton F. Fillius*  
*R. Frank Smith*  
ATTORNEYS

## UNITED STATES PATENT OFFICE

2,360,216

SUBBING PHOTOGRAPHIC PAPER  
SUPPORTS

Milton F. Fillius, Rochester, N. Y., assignor to  
Eastman Kodak Company, Rochester, N. Y., a  
corporation of New Jersey

Application June 8, 1943, Serial No. 490,039

6 Claims. (Cl. 95—9)

This invention relates to water-resistant photographic paper and to a method for subbing such paper.

In Bryce and Staehle U. S. application Serial No. 490,050, filed concurrently herewith, there is described a method for coating photographic paper with acrylate resins to render the paper moisture-resistant so that the paper does not absorb a large amount of water or chemicals during processing or during storage in changing atmospheric conditions. I have found that when a sensitive gelatin emulsion is coated on such resin coated paper the emulsion does not adhere well when the paper is wet, as during photographic processing.

It is, accordingly, an object of the present invention to provide a method for subbing resin coated photographic paper. A further object is to provide a method for preventing wet stripping of a photographic emulsion from resin coated photographic paper.

These objects are accomplished, according to my invention, by subbing the resin coated paper with a mixture of an acrylate resin and gelatin.

In the accompanying drawing, Fig. 1 is a sectional view of a resin coated paper having a single subbing layer according to my invention. Fig. 2 is a sectional view of a resin coated paper having two subbing layers of successively increasing gelatin content.

According to the invention described in the Bryce and Staehle U. S. application Serial No. 490,050, photographic paper is coated on both sides with a water suspension of a polyacrylate resin. The polyacrylate suspension may consist of the polymerization product of any of the usual acrylates well known in the industry such as acrylic acid, methyl acrylate, ethyl acrylate, acrylic acid nitrile, or mixtures of these in any proportions.

A photographic emulsion coated on the acrylate coated sheet will adhere fairly well when dry, but when wetted will separate from the acrylate coating. To overcome this, it is necessary to coat the acrylate coated sheet with a primer or sub and, for this purpose I have found that a mixture of the acrylate suspension and a gelatin solution to which formaldehyde or a chromium salt has been added works very well. The ratio of gelatin to acrylate which gives the most satisfactory result, varies depending upon the hardness of the acrylate used. I have found in practice that ratios varying from one part of gelatin in from  $\frac{1}{2}$  to 8 parts of acrylate resin is satisfactory. The use of the gelatin hardening agents mentioned above is optional since good results can be obtained in the absence of these agents.

The adhesion of the final sensitive emulsion can

be increased even further by the use of several subbing layers, in which the ratio of gelatin to acrylate is successively increased. This gradually changes the nature of the material from a 5 100% acrylate phase through several different ratios of the two common phases to a phase in which the adhesive material is 100% gelatin.

It has also been found that increased adhesion 10 of the final photographic emulsion to the support can be obtained by adding an acrylate resin to the emulsion. The amount of acrylate in the emulsion may vary from  $\frac{1}{4}$  the weight of the gelatin to about 3 times the weight of the gelatin in the emulsion. More or less acrylate may, however, be added to the emulsion.

In the accompanying drawing, Fig. 1 illustrates 15 a resin coated paper subbed according to my invention. As shown therein the support 10 is coated on both sides with layers 11 of an acrylate resin in the manner described in the Bryce and Staehle application Serial No. 490,050. The coating on the rear surface of the support may contain a wax as described in Vogel U. S. application Serial No. 490,049, filed concurrently herewith. One of the acrylate layers is coated with a subbing layer 12 of a dispersion of acrylate resin containing gelatin. After drying, this layer is 20 coated with the usual gelatino-silver halide emulsion layer 13.

Fig. 2 illustrates another modification of my 25 invention in which the paper support 10 is coated with the acrylate resin layers 11 and one of these layers is coated with successive subbing layers 14 and 15. The layer 14 contains a low amount of gelatin and a high amount of acrylate resin and the layer 15 contains a high amount of gelatin and a low amount of acrylate resin. The sensitive emulsion layer 13 is then coated 30 on layer 15. In this way the gelatin content of the successive layers is increased from the support outward so that good adhesion of the layers is obtained during and after photographic processing. It will be apparent that more than two 35 subbing layers may be applied, the proportion of gelatin to resin increasing in the successive layers.

40 My invention will be further illustrated by reference to the following specific examples.

## Example 1

A baryta-coated paper was coated on the baryta side with an aqueous dispersion of a polyacrylate resin containing 25% resin. On the opposite side 45 of the paper was coated an aqueous dispersion of a mixture of equal parts of a 25% aqueous dispersion of a polyacrylate resin and a 15% aqueous dispersion of carnauba wax. Over the first coating was applied a sub from a water system containing 3.5 parts of gelatin and 10 parts of polyacrylate resin in suspension. When dry, this

gave a layer containing three parts of acrylate resin and one part of gelatin. Over this was applied a sensitive gelatino-silver halide emulsion.

*Example 2*

Baryta-coated paper was coated on one side with a dispersion of a mixture of three parts of 25% polyacrylate resin dispersion and one part of 15% carnauba wax dispersion. After drying, the opposite side of the paper was coated with a 25% aqueous dispersion of a polyacrylate resin followed by a gelatin-resin sub-containing 10% polyacrylate resin and 3.5% gelatin which, on drying, gave a layer containing three parts of resin and one part of gelatin. This was followed by the usual photographic emulsion layer.

*Example 3*

Baryta-coated paper was coated on both sides with a 25% aqueous dispersion of a polyacrylate resin and the baryta side of the paper was then coated with a subbing layer from a dispersion of a mixture of one part of 3% gelatin solution and one part of 6% aqueous dispersion of a polyacrylate resin followed by the emulsion layer.

*Example 4*

Baryta-coated paper was coated on the rear surface with two separate layers each coated from a dispersion containing 3 parts of 25% aqueous dispersion of a polyacrylate resin and one part of a 15% aqueous dispersion of carnauba wax. On the baryta side was coated a 25% aqueous dispersion of a polyacrylate resin followed by a subbing layer coated from a mixture of one part of 8% polyacrylate resin dispersion and one part of 2% gelatin solution, followed by the emulsion layer.

*Example 5*

Baryta-coated paper was coated on both sides of a 25% aqueous dispersion of a polyacrylate resin and on the baryta side with a mixture of equal parts of 4% gelatin solution and a 5% aqueous dispersion of a polyacrylate resin. The latter coating was dried and coated with the usual sensitive emulsion layer.

*Example 6*

A baryta-coated paper was coated on the rear surface with a 25% aqueous dispersion of a medium hardness acrylate resin. The baryta-coated surface was coated with the same acrylate resin dispersion followed by two subbing layers, the first of which consisted of an aqueous dispersion of three parts of medium hardness acrylate resin and one part of gelatin and the second of which contained one part of the acrylate resin and three parts of gelatin. The paper was then coated with a photographic emulsion. Tests showed the paper to be highly water-resistant and satisfactory with respect to wet and dry adhesion.

*Example 7*

A baryta-coated paper base was coated on the rear surface with a 25% aqueous dispersion of a medium hardness acrylate resin to which one part of carnauba wax had been added. The baryta-coated surface was coated with a 25% aqueous dispersion of a medium hardness acrylate resin followed by a subbing layer of a dispersion of three parts of a soft polyacrylate resin to one part of gelatin. The paper was then coated with various photographic emulsions to which different amounts of a soft polyacrylate resin had been

added. Three coatings were made in which the ratio of acrylate resin to gelatin varied as follows: 1 to 4, 1 to 2 and 2 to 3. In all cases good, wet and dry adhesion and satisfactory water-resistance were obtained.

The acrylate resin used in the preparation of the sub according to my invention may consist of the polymerization product of any of the usual acrylates well known in the industry such as 10 acrylic acid, methyl acrylate, ethyl acrylate, acrylic acid nitrile, or mixtures of these in any proportions. I may use an aqueous dispersion such as that sold by the Rohm & Haas Chemical Corporation of Philadelphia, Pa., under the name Rhoplex W-66, which is believed to be a dispersion in water of a resin consisting principally of polymethyl acrylate and containing about 25% resin.

It will be understood that the examples and 20 modifications included herein are illustrative only and that my invention is to be taken as limited only by the scope of the appended claims.

I claim:

1. A light-sensitive photographic element having a water-resistant support, comprising a paper base coated on both sides thereof with a water-resistant acrylate resin, at least one of said acrylate resin layers being coated with a subbing layer comprising a mixture of an acrylate resin and gelatin, followed by a sensitive photographic emulsion layer.
2. A light-sensitive photographic element having a water-resistant support comprising a paper base coated on both sides thereof with a water-resistant acrylate resin, one of said acrylate resin layers being coated with at least two subbing layers comprising a mixture of an acrylate resin and gelatin, the proportion of gelatin to resin being successively increased in the layers farthest from the paper base, and the subbing layers being followed by a sensitive photographic emulsion layer.
3. A light-sensitive photographic element having a water-resistant support comprising a paper base coated on both sides thereof with a water-resistant acrylate resin, one of said acrylate resin layers being coated with a mixture of a subbing layer of acrylic acid ester resin and hardened gelatin, said subbing layer being coated with a sensitive photographic emulsion layer.
4. A light-sensitive photographic element having a water-resistant support comprising a paper base coated on both sides thereof with a water-resistant acrylate resin, one of said acrylate resin layers being coated with a subbing layer comprising a mixture of an acrylate resin and hardened gelatin, the ratio of gelatin to acrylate resin varying from one part of gelatin in from  $\frac{1}{2}$  to 8 parts of acrylate resin, said subbing layer being coated with a sensitive photographic emulsion layer.
5. The method of subbing a resin-coated photographic paper support, which comprises applying to said resin-coated support an aqueous dispersion of an acrylate resin containing gelatin, drying the coating thus formed, and applying thereto a sensitive gelatin emulsion layer.
6. The method of subbing a resin-coated photographic paper support, which comprises applying to said resin-coated support an aqueous dispersion of a polymethyl acrylate resin containing gelatin, drying the coating thus formed, and applying thereto a sensitive gelatin emulsion layer.

MILTON F. FILLIUS.